

# UNITED STATES PATENT OFFICE.

CHARLES T. MALCOLMSON, OF CHICAGO, ILLINOIS.

## BRIQUET.

1,012,676.

Specification of Letters Patent. Patented Dec. 26, 1911.

No Drawing.

Application filed January 10, 1910. Serial No. 537,168.

*To all whom it may concern:*

Be it known that I, CHARLES T. MALCOLMSON, a citizen of the United States, residing at Chicago, Illinois, have invented a certain 5 new and useful Improvement in Briquets, of which the following is a full, clear, and exact description, such as will enable others skilled in the art to which it appertains to make and use the same.

10 This invention relates to a new and useful improvement in the manufacture of briquets, the object being to produce a briquet having a dense compact body with a minimum amount of pitch or like binder.

15 Immense quantities of fine anthracite coal dust (culm) obtained in the preparation of "sized" anthracite coal for market, are piled as refuse near the mines. Usually this culm contains too much deleterious or non-

20 combustible matter to warrant its use commercially, so that when these culm banks are worked over to obtain the larger sizes contained in them, the coal is washed or jigged to remove part of the impurities.

25 The same process is used in the preparation of commercial sizes of anthracite at many of the mines to-day, making salable the hitherto unavailable small sizes such as "barley," "rice," etc. These smaller sizes are

30 not suited to domestic use, but are sold for steam purposes in the eastern cities, or burned on the locomotives of the anthracite carrying railroads, usually mixed with other coals.

35 In the middle and far west large lignite bearing areas exist. The better grade of this fuel is mined and sold for domestic and heating purposes, when higher grade coals are not available or are sold at such 40 a high price that the lignites can be sold in competition and bring a reasonable profit to the producer. These lignitic coals produce considerable slack in mining, which on account of its low fuel value and the fact 45 that it deteriorates rapidly when stored, is practically a waste product.

There are certain bituminous coals distributed throughout the country which will not produce coke. The slack from these 50 coals has no value except for steam purposes. There are processes developed in Europe by means of which "dry" coals, lignite and peat can be utilized in making gas and the resulting by-products find a 55 ready market. But in the United States the low price of fuels and excessive cost of

these plants has restricted their use. Briquetting plants are being established in this country for the utilization of these low grade or hitherto waste fuels. By this process the fine coal, "culm" or "slack" is mixed with a bonding material and compressed into "briquets" of various shapes and weighing from 2 ounces to 20 pounds. Briquetted coal produces results equal to or greater than lump coal from the same mine. 60

In general practice hard pitch made from coal or water gas tar is the binder used in briquetting coal. The percentage of pitch required to make satisfactory commercial 70 briquets varies with the size of briquet, character of the coal and process used. In making briquets from anthracite coal from 10 to 13 per cent. of pitch is used: briquets made from coking bituminous coal require 75 from 6 to 8 per cent., while in the briquetting of non-coking and semi-anthracite coals from 8 to 10 per cent. of hard pitch binder is used in commercial plants. As the binder is the largest item of cost, it is essential in 80 the interests of economical operation that the percentage be reduced to a minimum. Pitch is composed largely of volatile hydrocarbons or the smoke producing elements of coal. Thus it is desirable to add as little 85 pitch as possible in briquetting bituminous coals already high in volatile matter. In the treatment of anthracite and "lean" coals this feature is not objectionable.

Anthracite, the non-coking bituminous 90 coals, sub-bituminous coals and lignites have no coking or caking property: that is, briquets made from these coals will disintegrate rapidly during combustion unless the bonding material, with which 95 they are made, does not burn away faster than the coal in the briquet or remains unaffected at the temperatures necessary to the combustion of the coal. Pitch forms of itself a "coke" during combustion which is practically pure carbon and therefore burns at approximately the same rate as the "fixed carbon" of the coal; but the "coke" thus obtained is less than one-half 100 the mass of the original pitch and is a much inferior bonding agent.

By the addition, under pressure, of the necessary hydrocarbons contained in coal tar pitch, certain non-coking coals can be made 110 to produce coke; but in case of anthracite this consideration may be eliminated, and it becomes necessary to add an amount of pitch

in excess of that required to manufacture good briquets, in order that the coke formed during combustion will serve to hold the slower burning coal together until consumed.

- 5 An excessive amount of pitch is required to make briquets from raw lignite and sub-bituminous coals, for reasons explained below. It is also difficult to maintain the integrity of the briquets during combustion 10 owing to the excessive moisture contained in the coal which causes rapid "sparking" as the imprisoned water is transformed into steam.

The percentage of pitch required to make 15 a perfect bond depends on the amount of surface to be coated and the density of the coal. The surface depends on the size of the grains of coal and the number of their capillary pores. In other words, the amount of surface 20 varies inversely with the density of the coal and the diameter of the grains. Thus it has been shown, that while a coal of density 1.4 requires 6 per cent. of pitch to make a good briquet, a coal with density 1.1 requires 25  $7\frac{1}{2}$  per cent. of pitch to make a briquet equally good, all other conditions being the same. But the size of the grains is of more importance. It has been shown that the percentage 30 of voids for grains of uniform size is independent of the size of the grain, and is at its maximum, about 43 per cent., when the grains are uniform in size but irregular in shape. It is easily shown that pulverized coal which will just pass through a screen 35 with 20 meshes to the inch has 6.35 times the surface to be coated as that presented by an equal weight of coal passed through a screen with 4 meshes to the inch.

Exhaustive experiments have shown that 40 the cohesion or strength of the briquet begins with 4 per cent. of pitch and increases until 9 per cent. of binder is used, after which the cohesion of the briquet decreases until with 28 per cent. of binder the briquet equals that 45 of the pitch. Well made briquets have a greater cohesion than the coal or pitch from which they are made.

Washing anthracite, in the preparation of 50 small sizes, not only reduces the foreign substance or ash, but also takes away the very fine dust, leaving the small coal uniform in size and free from "fines."

A briquet must be dense in order to reduce 55 breakage in handling, to prevent the absorption of moisture (hygroscopic) and prevent excessive smoke during combustion. A dense briquet is obtained by filling the voids and manufacturing under high pressure. Either one of these factors may be varied at the expense of the other. In the fabrication of 60 small briquets the relatively large surface with relation to the volume makes possible a high total pressure on the surface of the briquet. But as the volume increases, in order 65 to maintain a constant ratio of mass and

pressure, the pressure per square inch of surface must increase at a much greater rate than the volume; this pressure soon becomes prohibitive for commercial plants. To overcome this deficiency the quantity of binder 70 is increased, in practice. Larger briquets are more economical from the consumers' standpoint, and therefore more desirable for house heating furnaces, locomotives or wherever it is desirable to maintain a deep fuel 75 bed.

It is essential that the binder be distributed uniformly through the coal in order that each particle shall become effective. In practice it is necessary to add sufficient binder 80 so that the minimum amount contained in any unit mass shall be equal to that necessary to make good briquets. This means that if the binder is not thoroughly mixed with the coal an excess of binder is necessary. 85

The difficulties attendant on making a perfect mixture of coal and binder in a commercial plant increase with a decrease in the percentage of binder used. Thus it is much 90 easier to mix 25 per cent. of binder and 75 per cent. of coal than 6 per cent. binder and 94 per cent. coal. The finer the binder is divided the easier it is to distribute it uniformly throughout the mass of coal. 95

We will consider here only the use of hard dry pitch as a binder and not the process by which the pitch is melted independently and introduced into the coal as a liquid. Even very hard pitch is difficult to grind or pulverize by mechanical means, and if the reduction is very fine, it is practically impossible to convey, store or measure it mechanically. The powdered pitch sticks to the machinery, and tends to return to a solid mass 100 if allowed to stand or if subjected to pressure or rubbing surfaces. The addition of coal to the pitch entirely eliminates these difficulties.

In the treatment of anthracite small sizes 110 with which we are particularly concerned, it is difficult and therefore expensive to reduce to "fines" the already minute and uniform grains of "barley" or "rice" by the use of "mills" or "pulverizers" available in the market today. The hammer type of crushers in general use depend upon the impact of a blow to break up the coal, and their effectiveness decreases rapidly with these small sizes. 115

In the formation of briquets according to my invention, I utilize fine hard anthracite particles of available sizes and fill the voids with a mixture of bituminous coking coal and pitch. 120

In the briquetting of anthracite coal in practice, I determine first the percentage of voids which we will assume to be 25 per cent. of the total volume of the coal. I then prepare the mixture of bituminous coking 125 coal and pitch. 130

coal and pitch in the right proportion, say 25 per cent. of pitch and 75 per cent. coking coal, having a total volume equal to the voids in the coal to be briqueted. This mixture of coking coal and pitch which we will call the "binder" is pulverized very fine and then thoroughly mixed with the coal. The mass is heated with the proper admixture of moisture to a temperature which will thoroughly liquefy the pitch after which it is cooled to a temperature at which the agglomerate can be successfully briqueted, passed through a briquetting press and molded into masses of definite size and shape. By this means I utilize a coal which will not detract, in any way, from the quality of the anthracite briquets, but one which can be easily reduced to the proper size to furnish the necessary fines to fill the voids, thus making the densest possible briquet under minimum pressure and with the minimum requirement of pitch. The addition of the coking coal not only reduces the percentage of binder necessary to make mechanically perfect briquets, but serves to hold the briquets together in the fire, and supply the volatile hydrocarbons essential to a high grade steam coal. The briquets will burn entirely from the surface, be retained as a compact mass after the volatile hydrocarbons of the pitch are driven off, and not disintegrate in the fire until entirely consumed.

In the case of coking and non-coking bituminous coals and sub-bituminous coals and lignites, my process serves to reduce the percentage of binder by a more even distribution of the pitch and a means of maintaining the proper percentage of fines to keep the voids at a minimum. With these coals my invention contemplates the use of

particles of coal not to exceed  $\frac{1}{4}$  inch in diameter, in combination with smaller sizes in the proper proportion to reduce to a minimum, the percentage of voids, and the total surface contained in the briquet. With lignites I am able to produce briquets which overcome largely the difficulties encountered in the use of raw lignite. The briquets will burn similarly to those made from bituminous coal, maintaining a coherent mass until entirely consumed. They will not be hygroscopic nor disintegrate when exposed to the weather. The characteristic "sparking" will be retarded if not entirely eliminated, and the objectionable "sparks" or cinders greatly reduced.

I claim:

1. A briquet composed essentially of hard anthracite particles, whose voids are filled with a composition of pulverized bituminous coking coal and pitch mixed to serve as a binder.
2. A briquet composed of anthracite coal particles, pulverized pitch mixed with bituminous coking coal particles, said mixture being heated until the pitch liquefies, and then cooled to a proper temperature for molding in a press.
3. A briquet composed of anthracite coal particles and a binder comprising pulverized pitch mixed with bituminous coal particles, the mixture of anthracite coal and binder being heated until the pitch liquefies.

In testimony whereof I hereunto affix my signature in the presence of two witnesses, this 8th day of January, 1910.

CHARLES T. MALCOLMSON.

Witnesses:

F. R. CORNWALL,  
M. P. SMITH.